# EUROPEAN PATENT SPECIFICATION

(11) **EP 0 883 736 B1**
(45) Date of publication and mention of the grant of the patent: **26.04.2000**
(21) Application number: 97905225.5
(22) Date of filing: 20.02.1997
(51) Int. Cl.: F01N 3/02, F01N 3/28, D04H 1/64

(54) **COMPOSITE FIBRE PRODUCTS AND PROCESSES FOR THEIR PRODUCTION**
FASERVERBUNDWERKSTOFFE UND VERFAHREN ZU IHRER HERSTELLUNG
PRODUITS FIBREUX COMPOSITES ET LEURS PROCEDES DE FABRICATION

(30) Priority: 27.02.1996 GB 9604097; 26.07.1996 GB 9615770
(43) Date of publication of application: 16.12.1998
(73) Proprietor: Saffil Limited, Sheffield, South Yorkshire S10 3GB (GB)
(72) Inventor: BOFFEY, Stuart Samuel, Crewe, Cheshire CW1 3AQ (GB); ASHER, Paul Martin Lawford, Tarvin, Chester CH3 8EY (GB)
(74) Representative: Shaw, Laurence
(86) International application number: GB9700466
(87) International publication number: WO9732118

(56) References cited:
- EP-A- 0 765 993
- WO-A-94/24425
- US-A- 4 011 651
- US-A- 5 580 532

## Description

The present invention relates to composite fibre products comprising a plurality of inorganic fibres which are bound together with a binder and to processes for their production. More particularly, the present invention relates to composite fibre mats which can be used for resiliently mounting the fragile ceramic or metal monoliths which are found in catalytic converters and diesel particulate filters in a surrounding metal casing.

Catalytic converters and diesel particulate filters are routinely fitted to automobiles and other road going vehicles in order to purify the exhaust gases which are generated by the engine. These devices usually comprise a ceramic honeycomb monolith which is housed within a metal casing and provides a support for the catalyst. The ceramic monolith comprises a plurality of tiny flow channels and is a fragile structure which is susceptible to damage when subjected to the kind of vibrational forces which prevail when any road going vehicle is in use. Moreover, the monolith and the surrounding metal casing are subjected to extremely high temperatures in use which causes them to expand, but not to the same extent. In consequence, the mounting system which is used to mount the ceramic monolith in its metal casing must insulate the monolith from the attendant vibrational forces and compensate for any difference between the expansion of the monolith and the casing. In this way, the stresses to which the monolith is subjected during use as a result of differential expansion or vibrational forces can be maintained at an acceptable level.

It is known to use a composite fibre mat to resiliently mount the fragile ceramic monolith which is found in catalytic converters and diesel particulate filters in a surrounding metal casing, see for example US-4,011,651 and WO-94/24425. The fibre mat is arranged in the annular space between the monolith and the surrounding metal casing and is maintained under compression in the annular space so exerting a radial pressure on the monolith and the casing which retains the monolith in place.

The present invention provides a composite fibre product comprising a plurality of inorganic fibres and a binder and a process for its production. The composite fibre product can take the form of a flexible mat which can be used to mount ceramic or metal monoliths found in catalytic converters and diesel particulate filters in their metal casings.

According to a first aspect of the present invention there is provided a composite fibre product, particularly a mat, which comprises a plurality of inorganic fibres and a binder which is substantially uniformly distributed throughout the fibre product, said composite fibre product having a laminar shear strength of at least 0.1 MPa.

The inorganic fibres may be any of the inorganic fibres known in the art. However, when the composite fibre product is a mat which is to be used for resiliently mounting the ceramic or metal monoliths contained in catalytic converters and diesel particulate filters, the fibres will need to be thermally stable (i.e. will not degrade) at the high operating temperatures prevailing in such devices. Typically, the fibres contained in composite fibre mats which are to be used in such mounting applications will be thermally stable at temperatures in excess of 700°C, preferably in excess of 800°C and more preferably in excess of 900°C.

Thermally stable inorganic fibres include ceramic fibres such as alumina, mullite, aluminosilicate, aluminoborosilicate, zirconia and titania fibres as well as vitreous glass fibres. The preferred thermally stable inorganic fibres are polycrystalline inorganic fibres, particularly polycrystalline inorganic oxide fibres, such as alumina, mullite, aluminosilicate, aluminoborosilicate, zirconia and titania fibres. Of these, alumina fibres, by which term we are also intending to include alumina fibres comprising a few weight % of silica added as a phase stabiliser, are particularly preferred. The fibres are preferably short staple fibres having a length in the range of from 1 to 10 cms and a mean diameter in the range of from 1 to 10 microns. Especially preferred alumina fibres are those sold in the form of a loosely bound, low density mat by Imperial Chemical Industries PLC under the trade name Saffil which are thermally stable at temperatures in excess of 1000°C.

The composite fibre products of the invention may comprise two or more different types of inorganic fibre. In this embodiment, the different fibre types may be intimately mixed or they may be segregated and arranged in definite patterns, e.g. in discrete layers.

The binder may be an inorganic material, but is preferably organic. Suitable organic binders are more particularly described in US-4,011,651 and WO-94/24425. Preferably the binder is an organic polymer.

One suitable binder is a copolymer based on n-butyl acrylate and acrylonitrile.

Preferred binders are those obtained on curing a curable polymer composition. Preferred examples of curable polymer compositions are those comprising a combination of an acrylic polymer and a cross-linking agent, particular an epoxy group containing cross-linking agent such as an epoxy resin. Curable polymer compositions of this type will typically comprise from 90.0 to 99.0 % by weight, preferably from 95.0 to 99.0 % by weight of the acrylic polymer and from 1.0 to 10.0 % by weight, preferably from 1.0 to 5.0 % by weight of the cross-linking agent. The acrylic polymer is suitably a homopolymer or copolymer comprising monomer units derived from at least one acrylic monomer selected from the C₁₋₈ alkyl (C₁₋₄ alkyl)acrylates, and in a preferred embodiment is a homopolymer or copolymer comprising monomer units derived from at least one acrylic monomer selected from the C₁₋₄ alkyl (meth)acrylates, for example methyl methacrylate, methyl acrylate, ethyl acrylate, propyl acrylate and butyl acrylate. An especially preferred binder is that obtained on curing a composition comprising an acrylic polymer based on butyl acrylate and an epoxy resin cross-linking agent.

When a composite fibre mat of the invention is to be used for mounting a ceramic or metal monolith in a catalytic converter or in a diesel particulate filter, it is preferred to use an organic binder which will be substantially pyrolysed/burned out by the high temperatures to which the mat will be subjected in use. In addition, the organic binder is preferably one which will not lead to the generation of toxic emissions when it is pyrolysed/burned out and for this reason is preferably free of chlorine and nitrogen.

The binder contained in the composite fibre product of the present invention is substantially uniformly distributed throughout the fibre product. Preferably the distribution of the binder in the composite fibre product is such that the percentage by weight of binder in each 1 mm³ region of the product based on the total weight of the product in that region is within 40 %, more preferably within 30 % and particularly preferably within 20 % of the overall percentage by weight of binder in the product based on the total weight of the product. In an especially preferred embodiment, the distribution of the binder in the composite fibre product is such that the percentage by weight of binder in each 1 mm³ region of the product based on the total weight of the product in that region is within 10 % of the overall percentage by weight of binder in the product based on the total weight of the product.

The thickness of the composite fibre product will depend on the intended end use for the product. However, when the product is a composite fibre mat for mounting a ceramic or metal monolith in a catalytic converter or in a diesel particulate filter, it will typically have a thickness in the range of from 3 to 15 mm, preferably in the range of from 5 to 12 mm and more preferably in the range of from 5 to 9 mm.

The loading of the binder in the composite fibre product will typically be in the range of from 2 to 15 % by weight and preferably in the range of from 5 to 15 % by weight based on the total weight of the product.

The composite fibre product of the invention typically has a density in the range of from 30 to 700 kg/m³, preferably in the range of from 100 to 500 kg/m³ and more preferably in the range of from 100 to 350 kg/m³.

The composite fibre product of the invention has a laminar shear strength, by which is meant the force which has to be applied in order to bring about delamination of the product, of at least 0.1 MPa, preferably of at least 0.2 MPa and more preferably of at least 0.3 MPa. The laminar shear strength can be conveniently measured on an Instron or similar machine using a three point bend test. Preferably the composite fibre product is also capable of exerting a pressure of at least 1.0 kgf/cm², more preferably in the range of from 1.5 to 4.0 kgf/cm² when a sample of the product having a thickness in the range of from 5 to 10 mm is compressed to a thickness of 3 mm between two plates and the binder removed.

According to a second aspect of the present invention there is provided a process for the production of a composite fibre product, particularly a mat, which comprises impregnating a fibre mass comprising a plurality of inorganic fibres with a liquid binder system comprising a binder material and a carrier liquid and subjecting the impregnated fibre mass to a heating step,
characterised in that the heating step involves the use of dielectric heating, such as microwave or radio frequency heating. In this second aspect of the present invention, the impregnated fibre mass is preferably held under compression during at least a part of the heating step.

The fibre mass which is impregnated in the processes of the present invention may comprise a plurality of discrete fibres or it may take the form of a multi-fibre product in which the individual fibres are assembled into a low density mat or blanket which is loosely held together by fibre intertwining or perhaps more robustly consolidated by some other means such as weaving, knitting,
stitching, needle-punching or vacuum packing. Preferably the fibre mass which is impregnated in the processes of the present invention is a multi-fibre product having a thickness in the range of from 10 to 60 mm, more preferably in the range of from 30 to 50 mm, and an area density in the range of from 0.2 to 2.0 kg/m², more preferably in the range of from 1.0 to 2.0 kg/m². The inorganic fibres and preferred inorganic fibres for use in the processes of the present invention are as described previously in connection with the composite fibre product.

The processes of the present invention may be used to prepare composite fibre products from two or more different types of inorganic fibre. In this embodiment, the different fibre types may be intimately mixed or they may be segregated and arranged in definite patterns, e.g. in discrete layers.

The liquid binder system may comprise an inorganic binder material, but preferably comprises an organic binder material, such as a polymer, and an organic or aqueous carrier liquid which is able to dissolve or disperse the organic binder material. Suitable organic binder materials are more particularly described in US-4,011,651 and WO-94/24425, the disclosures in which are incorporated herein by way of reference, and include polymers as well as curable polymers or prepolymers which can be cured in situ on the impregnated fibre mass as part of the drying step or in a subsequent processing step. The polymer may be a material which allows for the recovery of fibres from waste product generated in a process of the present invention or in subsequent processing/finishing operations.

One suitable binder system comprises an aqueous dispersion of a copolymer based on n-butyl acrylate and acrylonitrile.

Preferred binder systems are those comprising a dispersion, preferably an aqueous dispersion, of a curable polymer composition, sometimes termed a resin or latex. Examples of preferred curable polymer compositions are those comprising a combination of an acrylic polymer and a cross-linking agent, particular an epoxy group containing cross-linking agent such as an epoxy resin. Curable polymer compositions of this type will typically comprise from 90.0 to 99.0 % by weight, preferably from 95.0 to 99.0 % by weight of the acrylic polymer and from 1.0 to 10.0 % by weight, preferably from 1.0 to 5.0 % by weight of the cross-linking agent. The acrylic polymer is suitably a homopolymer or copolymer comprising monomer units derived from at least one acrylic monomer selected from the C₁₋₈ alkyl (C₁₋₄ alkyl)acrylates, and in a preferred embodiment is a homopolymer or copolymer comprising monomer units derived from at least one acrylic monomer selected from the C₁₋₄ alkyl (meth)acrylates, for example methyl methacrylate, methyl acrylate, ethyl acrylate, propyl acrylate and butyl acrylate. An especially preferred binder system is one comprising an aqueous dispersion of an acrylic polymer based on butyl acrylate and an epoxy resin cross-linking agent.

When the liquid binder system is one comprising a curable polymer composition, it may also comprise a catalyst to accelerate the curing process.

It will be appreciated from the above, that by the term liquid binder system we are also intending to include binder systems which comprise dispersions or suspensions of finely divided solids in liquid vehicles.

The liquid binder system will typically comprise from 0.5 to 50.0 % by weight of the binder material and from 50.0 to 99.5 % by weight of the carrier liquid. Preferably the liquid binder system will comprise from 0.5 to 10.0 % by weight, more preferably from 1.0 to 5.0 % by weight of the binder material and from 90.0 to 99.5 % by weight, more preferably from 95.0 to 99.0 % by weight of the carrier liquid.

Various techniques may be used to impregnate the mass of inorganic fibres. For example, the individual fibres may be thoroughly dispersed in the liquid binder system and the resulting dispersion cast into sheets using a paper making process which involves removing excess carrier liquid, e.g. by vacuum.
Alternatively, where the mass of inorganic fibres takes the form of a multi-fibre product in which the individual fibres are assembled into a low density mat or blanket, the mat or blanket may be simply immersed or soaked in the liquid binder system. Alternatively, the low density fibre mat may be sprayed with the liquid binder system.

Before the impregnated fibre mass is subjected to the drying/heating step, it will often be convenient to remove any excess carrier liquid. This can be achieved by pressing the impregnated fibre mass between rollers or plates, by placing it under vacuum or by centrifuging.

After the fibre mass has been impregnated with the liquid binder system, and generally following removal of any excess carrier liquid, the impregnated fibre mass is subjected to a drying/heating step. In the processes of the second and third aspects of the present invention and preferably also in the process of the fourth aspect of the present invention, at least a part of the drying/heating step is conducted while the impregnated fibre mass is held under compression. The impregnated fibre mass should be held under compression until such time as the binder material is able to hold the fibres together and significantly limit the expansion of the composite fibre product once the compressive forces are released. Generally, the whole of the drying/heating step will be performed while the impregnated fibre mass is held under compression, but it may be possible to perform just the final stages of the drying/heating step in this manner and still obtain satisfactory results. During the drying/heating step, substantially all and preferably all of any residual carrier liquid will be removed.

The pressure which is applied during the drying/heating step to compress the impregnated fibre mass will generally be in the range of from 5 to 500 KPa, preferably in the range of from 5 to 200 KPa. In general, the pressure applied is such as to produce a composite fibre product having a density in the range of from 30 to 700 kg/m³, preferably in the range of from 100 to 500 kg/m³, more preferably in the range of from 100 to 350 kg/m³. When the fibre mass which is impregnated is a multi-fibre product having a thickness in the range of from 10 to 60 mm, e.g. in the range of from 30 to 50 mm, and an area density in the range of from 0.2 to 2.0 kg/m², e.g. in the range of from 1.0 to 2.0 kg/m², the resulting impregnated fibre mass will generally be compressed to a thickness in the range of from 2 to 5 mm during the drying/heating step. This pressure is conveniently applied in a batch process by sandwiching the impregnated fibre mass between plates and then squeezing the plates together, e.g. by means of clamps, spring loaded clips or hydraulic presses. Alternatively, in a continuous process, it may be convenient to generate the necessary compressive forces on the impregnated fibre mass by feeding it through an arrangement of rollers or belts.

In the processes of the second and third aspects of the present invention, a conventional oven may be employed to carry out the drying/heating step, but in a preferred embodiment dielectric heating such as microwave or radio frequency heating is employed since it tends to result in an appreciably more uniform distribution of the binder in the final composite fibre product. In the processes of each of the second, third and fourth aspects of the present invention, it is preferred to use a combination of dielectric heating and a conventional heating means, such as a flow of hot air. Typically, the drying/heating step will involve heating the impregnated fibre mass to a temperature in the range of from 80 to 200°C, preferably in the range of from 100 to 170°C. Temperatures in the range of from 140 to 160°C are especially preferred.

When the liquid binder system comprises a curable polymer composition, as is preferred, the drying/heating step may be followed by a further processing step in which the curable polymer composition is cured. This curing process preferably involves the polymer composition undergoing some form of cross-linking reaction. However, the temperatures which are employed in the drying/heating step are usually sufficient to remove any residual carrier liquid and cure the curable polymer composition so that a separate curing step is generally unnecessary. When a separate curing step is employed, however, the impregnated fibre mass will generally be held under compression for the duration of the curing step.

The composite fibre product of the present invention may also contain one or more other materials. Suitable materials for inclusion in the composite fibre product include the layer minerals, particularly the expandable layer silicate minerals such as vermiculite. The incorporation of another material into the composite fibre product may be achieved by adding the material to a liquid binder system used in the preparation of such a product.

Alternatively, a composite fibre product prepared in accordance with the present processes may be post-treated with a solution or dispersion of the material to be incorporated.

Composite fibre products of the present invention may be used as mounting mats to mount ceramic and metal monoliths in catalytic converters and diesel particulate filters or to support the ceramic monoliths found in hot gas filtration units and coal gasification plants. Composite fibre products of the invention may also be usefully employed in gasket applications and as a high temperature insulation material.

The present invention is now illustrated but not limited with reference to the following examples.

### Example 1

Samples of "Saffil" low density mat having a size of about 500 mm by 200 mm were cut from a bulk product having a known area density of from 1.2 to 1.6 kg/m² and a thickness of from 30 to 50 mm. These samples were weighed and then transferred to a tray where they were soaked in a latex (Acronal 35D, a 50 % aqueous dispersion of a copolymer based on n-butyl acrylate and acrylonitrile available from BASF) which had been diluted to a solids content of around 3 % w/w. The impregnated samples were then sandwiched between two sheets of PTFE-coated glass fibre mesh and these sandwiches were then placed between two sheets of glass fibre filled silicone resin board of size 500 mm by 200 mm by 12 mm. The resin boards were then pressed together using G-clamps until the impregnated "Saffil" layers were reduced to a thickness of about 5 mm (equal to an applied pressure of about 0.5 bar (50 KPa)), and held in this position with clips. During this assembly excess latex drained from the samples.

The completed mould assemblies were then placed on the belt of an air/radio frequency (RF) assisted oven and the belt speed was adjusted to give a residence time of between 15 and 45 minutes. The RF power to the oven was set at about 5.5 KW and the temperature of the air in the oven was adjusted to about 150°C. The samples were removed from the oven when the latex had been fully dried and cured (cross-linked). The clips and the boards were then carefully removed from the samples and the PTFE mesh peeled off to reveal the final composite fibre mats which had a thickness in the range of from 7 to 8.5 mm.

### Example 2

Samples of "Saffil" low density mat having a size of about 500 mm by 200 mm were cut from a bulk product having a known area density of from 1.0 to 2.0 kg/m² and a thickness of from 30 to 50 mm. These samples were weighed and then transferred to a tray where they were soaked in a latex (60 % aqueous dispersion of a butyl acrylate based polymer containing 3 % w/w of Epikote (TM) 828 epoxy resin cross-linking agent) which had been diluted to a solids content of around 5 % w/w. The impregnated samples were then sandwiched between two sheets of PTFE-coated glass fibre mesh and these sandwiches were then placed between two sheets of glass fibre filled silicone resin board of size 500 mm by 200 mm by 12 mm. The resin boards were then pressed together using G-clamps until the impregnated "Saffil" layers were reduced to a thickness of about 5 mm (equal to an applied pressure of about 0.5 bar (50 KPa)), and held in this position with clips. During this assembly excess latex drained from the samples.

The completed mould assemblies were then placed on the belt of an air/radio frequency (RF) assisted oven and the belt speed was adjusted to give a residence time of between 15 and 45 minutes. The RF power to the oven was set at about 5.5 KW and the temperature of the air in the oven was adjusted to about 150°C. The samples were removed from the oven when the latex had been fully dried and cured (cross-linked). The clips and the boards were then carefully removed from the samples and the PTFE mesh peeled off to reveal the final composite fibre mats which had a thickness in the range of from 7 to 8.5 mm.

## Claims

1. A composite fibre product which comprises a plurality of inorganic fibres and a binder which is substantially uniformly distributed throughout the fibre product, said composite fibre product having a laminar shear strength of at least 0.1 MPa.

2. A composite fibre product as claimed in claim 1 wherein the inorganic fibres are thermally stable at temperatures in excess of 700°C.

3. A composite fibre product as claimed in claim 1 or claim 2 wherein the inorganic fibres are ceramic fibres.

4. A composite fibre product as claimed in claim 2 or claim 3 wherein the inorganic fibres are polycrystalline inorganic oxide fibres selected from the group consisting of alumina fibres, mullite fibres, aluminosilicate fibres, aluminoborosilicate fibres, zirconia fibres and titania fibres.

5. A composite fibre product as claimed in claim 4 wherein the inorganic fibres are alumina fibres.

6. A composite fibre product as claimed in any one of claims 1 to 5 wherein the inorganic fibres are short staple fibres having a length in the range of from 1 to 10 cms and a mean diameter in the range of from 1 to 10 microns.

7. A composite fibre product as claimed in any one of claims 1 to 6 wherein the binder is an organic material.

8. A composite fibre product as claimed in claim 7 wherein the binder is an organic polymer.

9. A composite fibre product as claimed in claim 7 or claim 8 wherein the binder is a material derived from curing a curable polymer composition comprising an acrylic polymer and an epoxy group containing cross-linking agent.

10. A composite fibre product as claimed in claim 9 wherein the acrylic polymer is a homopolymer or copolymer comprising monomer units derived from at least one acrylic monomer selected from the C₁₋₄ alkyl (meth)acrylates.

11. A composite fibre product as claimed in claim 9 wherein the binder is a material derived from curing a curable polymer composition comprising an acrylic polymer based on butyl acrylate and an epoxy resin cross-linking agent.

12. A composite fibre product as claimed in any one of the preceding claims wherein the distribution of the binder in the composite fibre product is such that the percentage by weight of binder in each 1 mm³ region of the product based on the total weight of the product in that region is within 40 % of the overall percentage by weight of binder in the product based on the total weight of the product.

13. A composite fibre product as claimed in claim 12 wherein the distribution of the binder in the composite fibre product is such that the percentage by weight of binder in each 1 mm³ region of the product based on the total weight of the product in that region is within 30 % of the overall percentage by weight of binder in the product based on the total weight of the product.

14. A composite fibre product as claimed in any one of the preceding claims which has a thickness in the range of from 3 to 15 mm.

15. A composite fibre product as claimed in any one of the preceding claims wherein the loading of the binder in the product is in the range of from 2 to 15 % by weight based on the total weight of the product.

16. A composite fibre product as claimed in any one of the preceding claims which has a density in the range of from 30 to 700 kg/m³.

17. A composite fibre product as claimed in claim 16 which has a density in the range of from 100 to 500 kg/m³.

18. A composite fibre product as claimed in any one of the preceding claims which has a laminar shear strength of at least 0.2 MPa.

19. A composite fibre product as claimed in any one of the preceding claims which is capable of exerting a pressure of at least 1.0 kgf/cm² when a sample of the product having a thickness in the range of from 5 to 10 mm is compressed to a thickness of 3 mm between two plates and the binder removed.

20. A composite fibre product as claimed in claim 19 which is capable of exerting a pressure in the range of from 1.5 to 4.0 kgf/cm² when a sample of the product having a thickness in the range of from 5 to 10 mm is compressed to a thickness of 3 mm between two plates and the binder removed.

21. A process for the production of a composite fibre product which comprises impregnating a fibre mass comprising a plurality of inorganic fibres with a liquid binder system comprising a binder material and a carrier liquid and subjecting the impregnated fibre mass to a heating step, characterised in that the heating step involves the use of dielectric heating.

22. A process as claimed in claim 21 wherein the impregnated fibre mass is held under compression during at least a part of the heating step.

23. A process as claimed in claim 21 or 22 wherein the fibre mass which is impregnated is a multi-fibre product in which the individual fibres are assembled into a low density mat or blanket.

24. A process as claimed in claim 23 wherein the multi-fibre product has a thickness in the range of from 10 to 60 mm and an area density in the range of from 0.2 to 2.0 kg/m².

25. A process as claimed in any one of claims 21 to 24 wherein the inorganic fibres are thermally stable at temperatures in excess of 700°C.

26. A process as claimed in claim 25 wherein the inorganic fibres are ceramic fibres.

27. A process as claimed in claim 25 or claim 26 wherein the inorganic fibres are polycrystalline inorganic oxide fibres selected from the group consisting of alumina fibres, mullite fibres, aluminosilicate fibres, aluminoborosilicate fibres, zirconia fibres and titania fibres.

28. A process as claimed in claim 27 wherein the inorganic fibres are alumina fibres.

29. A process as claimed in any one of claims 21 to 28 wherein the inorganic fibres are short staple fibres having a length in the range of from 1 to 10 cms and a mean diameter in the range of from 1 to 10 microns.

30. A process as claimed in any one of claims 21 to 29 wherein the liquid binder system comprises an organic binder material and an organic or aqueous carrier liquid which is able to dissolve or disperse the organic binder material.

31. A process as claimed in claim 30 wherein the organic binder material is a polymer.

32. A process as claimed in claim 30 or claim 31 wherein the liquid binder system comprises a dispersion of a curable polymer composition comprising an acrylic polymer and an epoxy group containing cross-linking agent.

33. A process as claimed in claim 32 wherein the acrylic polymer is a homopolymer or copolymer comprising monomer units derived from at least one acrylic monomer selected from the C₁₋₄ alkyl (meth)acrylates.

34. A process as claimed in claim 32 wherein the liquid binder system comprises a dispersion of a curable polymer composition comprising an acrylic polymer based on butyl acrylate and an epoxy resin cross-linking agent.

35. A process as claimed in any one of claims 30 to 34 wherein the dispersion is an aqueous dispersion.

36. A process as claimed in any one of claims 21 to 35 wherein the liquid binder system comprises from 0.5 to 50.0 % by weight of the binder material and from 50.0 to 99.5 % by weight of the carrier liquid.

37. A process as claimed in claim 36 wherein the liquid binder system comprises from 1.0 to 5.0 % by weight of the binder material and from 95.0 to 99.0 % by weight of the carrier liquid.

38. A process as claimed in claim 22 wherein the whole of the drying/heating step is performed while the impregnated fibre mass is held under compression.

39. A process as claimed in claim 22 wherein the pressure which is applied during the drying/heating step to compress the impregnated fibre mass is in the range of from 5 to 500 KPa.

40. A process as claimed in claim 39 wherein the pressure which is applied during the drying/heating step to compress the impregnated fibre mass is in the range of from 5 to 200 KPa.

41. A process as claimed in claim 21, wherein the dielectric heating means is microwave or radio frequency heating.

42. A process as claimed in claim 21, wherein a combination of dielectric heating and conventional heating is employed in the drying/heating step.

43. A process as claimed in any one of claims 21 to 42 wherein the impregnated fibre mass is heated to a temperature in the range of from 80 to 200°C in the drying/heating step.

44. A process as claimed in claim 43 wherein the impregnated fibre mass is heated to a temperature in the range of from 100 to 170°C in the drying/heating step.

## Patentansprüche

1. Faserkompositprodukt umfassend eine Vielzahl von anorganischen Fasern und ein Bindemittel, welches weitgehend gleichförmig über das Faserprodukt verteilt ist und das Faserkompositprodukt eine laminare Scherfestigkeit von wenigstens 0,1 MPa besitzt.

2. Faserkompositprodukt nach Anspruch 1, worin die anorganischen Fasern bei Temperaturen über 700°C thermisch stabil sind.

3. Faserkompositprodukt nach Anspruch 1 oder Anspruch 2, worin die anorganischen Fasern keramische Fasern sind.

4. Faserkompositprodukt nach Anspruch 2 oder Anspruch 3, worin die anorganischen Fasern polykristalline anorganische Oxidfasern sind, ausgewählt aus der Gruppe, bestehend aus Aluminafasern, Mullitfasern, Aluminosilikatfasern, Aluminoborosilikatfasern, Zirkoniumfasern und Titanfasern.

5. Faserkompositprodukt nach Anspruch 4, worin die anorganischen Fasern Aluminafasern sind.

6. Faserkompositprodukt nach einem der Ansprüche 1 bis 5, worin die anorganischen Fasern kurze Stapelfasern mit einer Länge im Bereich von 1 bis 10 cm und einem mittleren Durchmesser im Bereich von 1 bis 10 µm sind.

7. Faserkompositprodukt nach einem der Ansprüche 1 bis 6, worin das Bindemittel ein organisches Material ist.

8. Faserkompositprodukt nach Anspruch 7, worin das Bindemittel ein organisches Polymer ist.

9. Faserkompositprodukt nach Anspruch 7 oder Anspruch 8, worin das Bindemittel ein Material ist, abgeleitet vom Härten einer härtbaren Polymerzusammensetzung, umfassend ein Acrylpolymer und ein Epoxygruppe-enthaltendes Vernetzungsmittel.

10. Faserkompositprodukt nach Anspruch 9, worin das Acrylpolymer ein Homopolymer oder Copolymer ist, umfassend Monomereinheiten, abgeleitet von wenigstens einem Acrylmonomer, ausgewählt aus C₁₋₄ Alkyl(meth)acrylaten.

11. Faserkompositprodukt nach Anspruch 9, worin das Bindemittel ein Material ist, abgeleitet aus dem Härten einer härtbaren Polymerzusammensetzung, umfassend ein Acrylpolymer, basierend auf Butylacrylat, und ein Epoxyharz-Vernetzungsmittel.

12. Faserkompositprodukt nach einem der vorhergehenden Ansprüche, worin die Verteilung des Bindemittels in dem Faserkompositprodukt derart ist, daß der Gewichtsprozentsatz an Bindemittel in jedem 1 mm³ Bereich des Produkts, bezogen auf das Gesamtgewicht des Produkts in diesem Bereich, innerhalb 40% des gesamten Gewichtsprozentsatzes des Bindemittels im Produkt, bezogen auf das Gesamtgewicht des Produkts, liegt.

13. Faserkompositprodukt nach Anspruch 12, worin die Verteilung des Bindemittels in dem Faserkompositprodukt derart ist, daß der Gewichtsprozentsatz an Bindemittel in jedem 1 mm³ Bereich des Produkts, bezogen auf das Gesamtgewicht des Produkts in diesem Bereich innerhalb 30% des Gesamtgewichtsprozentsatzes an Bindemittel in dem Produkt, bezogen auf das Gesamtgewicht des Produkt, liegt.

14. Faserkompositprodukt nach einem der vorhergehenden Ansprüche, welches eine Dicke im Bereich von 3 bis 15 mm aufweist.

15. Faserkompositprodukt nach einem der vorhergehenden Ansprüche, worin die Beladung des Bindemittels im Produkt im Bereich von 2 bis 15 Gew.%, bezogen auf das Gesamtgewicht des Produkts, beträgt.

16. Faserkompositprodukt nach einem der vorhergehenden Ansprüche, welches eine Dichte im Bereich von 30 bis 700 kg/m³ aufweist.

17. Faserkompositprodukt nach Anspruch 16, welches eine Dichte im Bereich von 100 bis 500 kg/m³ aufweist.

18. Faserkompositprodukt nach einem der vorhergehenden Ansprüche, welches eine laminare Scherfestigkeit von wenigstens 0,2 MPa aufweist.

19. Faserkompositprodukt nach einem der vorhergehenden Ansprüche, welches fähig ist, einen Druck von wengistens 1,0 kgf/cm² auszuüben, wenn eine Produktprobe mit einer Dicke im Bereich von 5 bis 10 mm auf eine Dicke von 3 mm zwischen zwei Platten komprimiert wird und das Bindemittel entfernt wird.

20. Faserkompositprodukt nach Anspruch 19, welches fähig ist einen Druck im Bereich von 1,5 bis 4,0 kgf/cm² auszuüben, wenn eine Produktprobe mit einer Dicke im Bereich von 5 bis 10 mm auf eine Dicke von 3 mm zwischen zwei Platten komprimiert und das Bindemittel entfernt wird.

21. Verfahren zur Herstellung eines Faserkompositprodukts, umfassend Imprägnieren einer Fasermasse, umfassend eine Vielzahl von anorganischen Fasern, mit einem flüssigen Bindemittelsystem umfassend ein Bindemittelmaterial und eine Trägerflüssigkeit, und unterwerfen der imprägnierten Fasermasse einem Heizschritt, dadurch gekennzeichnet, daß der Heizschritt die Verwendung dielektrischer Heizung einschließt.

22. Verfahren nach Anspruch 21, worin die imprägnierte Fasermasse während wenigstens eines Teils des Heizschritts unter Druck gehalten wird.

23. Verfahren nach Anspruch 21 oder 22, worin die imprägnierte Fasermasse ein Multifaserprodukt ist, bei welchem die individuellen Fasern zu einer Matte oder eine Decke mit niedriger Dichte zusammengesetzt sind.

24. Verfahren nach Anspruch 23, worin das Multifaserprodukt eine Dicke im Bereich von 10 bis 16 mm und eine Flächendichte im Bereich von 0,2 bis 2,0 kg/m² aufweist.

25. Verfahren nach einem der Ansprüche 21 bis 24, worin die anorganischen Fasern bei Temperaturen oberhalb 700°C thermisch stabil sind.

26. Verfahren nach Anspruch 25, worin die anorganischen Fasern keramische Fasern sind.

27. Verfahren nach Anspruch 25 oder Anspruch 26, worin die anorganischen Fasern polykristalline anorganische Oxidfasern sind, ausgewählt aus der Gruppe, bestehend aus Aluminafasern, Mullitfasern, Aluminosilikatfasern, Aluminoborosilikatfasern, Zirkoniumfasern und Titanfasern.

28. Verfahren nach Anspruch 27, worin die anorganischen Fasern Aluminafasern sind.

29. Verfahren nach einem der Ansprüche 21 bis 28, worin die anorganischen Fasern kurze Stapelfasern mit einer Länge im Bereich von 1 bis 10 cm und einem mittleren Durchmesser im Bereich von 1 bis 10 µm sind.

30. Verfahren nach einem der Ansprüche 21 bis 29, worin das flüssige Bindemittelsystem ein organisches Bindemittelmaterial umfaßt und eine organische oder wässrige Trägerflüssigkeit, welche fähig ist, das organische Bindemittelmaterial zu lösen oder zu dispergieren.

31. Verfahren nach Anspruch 30, worin das organische Bindemittelmaterial ein Polymer ist.

32. Verfahren nach Anspruch 30 oder Anspruch 31, worin das flüssige Bindemittelsystem eine Dispersion aus einer härtbaren Polymerzusammensetzung umfaßt, umfassend ein Acrylpolymer und ein Epoxygruppe-enthaltendes Vernetzungsmittel.

33. Verfahren nach Anspruch 32, worin das Acrylpolymer ein Homopolymer oder Copolymer ist, umfassend Monomereinheiten, abgeleitet von wenigstens einem Acrylmonomer, ausgewählt aus den C₁₋₄ Alkyl(meth)acrylaten.

34. Verfahren nach Anspruch 32, worin das flüssige Bindemittelsystem eine Dispersion aus einer härtbaren Polymerzusammensetzung umfaßt, umfassend ein Acrylpolymer, basierend auf Butylacrylat, und ein Epoxyharz-Vernetzungsmittel.

35. Verfahren nach einem der Ansprüche 30 bis 34, worin die Dispersion eine wässrige Dispersion ist.

36. Verfahren nach einem der Ansprüche 21 bis 35, worin das flüssige Bindemittelsystem 0,5 bis 50,0 Gew.% Bindemittelmaterial und 50,0 bis 99,5 Gew.% Trägerflüssigkeit umfaßt.

37. Verfahren nach Anspruch 36, worin das flüssige Bindemittelsystem 1,0 bis 5,0 Gew.% Bindemittelmaterial und 95,0 bis 99,9 Gewichts% Trägerflüssigkeit umfaßt.

38. Verfahren nach Anspruch 22, worin der gesamte Trocknungs/Heizschritt durchgeführt wird, während die imprägnierte Fasermasse unter Kompression gehalten ist.

39. Verfahren nach Anspruch 22, worin der Druck, welcher während dem Trocknungs/Heizschritt angewandt wird, um die imprägnierte Fasermasse zu komprimieren, im Bereich von 5 bis 500 kPa liegt.

40. Verfahren nach Anspruch 39, worin der Druck, welcher während dem Trocknungs/Heizschritt angewandt wird, um die imprägnierte Fasermasse zu komprimieren, im Bereich von 5 bis 200 kPa liegt.

41. Verfahren nach Anspruch 21, worin die dielektrische Heizeinrichtung eine Mikrowellen- oder Radiofrequenzheizung ist.

42. Verfahren nach Anspruch 21, worin eine Kombination von dielektrischem Heizen und herkömmlichen Heizen während dem Trocknungs/Heizschritt verwendet wird.

43. Verfahren nach einem der Ansprüche 21 bis 47, worin die imprägnierte Fasermasse auf eine Temperatur im Bereich von 80 bis 200°C im Trocknungs/Heizschritt erhitzt wird.

44. Verfahren nach Anspruch 43, worin die imprägnierte Fasermasse auf eine Temperatur im Bereich von 100 bis 170°C im Trocknungs/Heizschritt erhitzt wird.

## Revendications

1. Produit en fibres composites qui comprend une pluralité de fibres inorganiques et un liant qui est réparti de façon très uniforme dans le produit en fibres, ledit produit en fibres composites ayant un cisaillement laminaire d'au moins 0,1 MPa.

2. Produit en fibres composites selon la revendication 1, dans laquelle les fibres inorganiques ont une stabilité thermique pour des températures supérieures à 700°C.

3. Produit en fibres composites selon la revendication 1 ou la revendication 2, dans laquelle les fibres inorganiques sont des fibres céramiques.

4. Produit en fibres composites selon la revendication 2 ou la revendication 3, dans laquelle les fibres inorganiques sont des fibres d'oxydes inorganiques polycristallins choisies dans le groupe constitué par les fibres d'alumine, les fibres de mullite, les fibres d'aluminosilicate, les fibres d'aluminoborosilicate, les fibres de zircone et les fibres de titane.

5. Produit en fibres composites selon la revendication 4, dans laquelle les fibres inorganiques sont des fibres d'alumine.

6. Produit en fibres composites selon l'une quelconque des revendications 1 à 5, dans laquelle les fibres inorganiques sont de courtes fibres discontinues ayant une longueur allant de 1 à 10 cm et un diamètre moyen allant de 1 à 10 microns.

7. Produit en fibres composites selon l'une quelconque des revendications 1 à 6, dans laquelle le liant est une substance organique.

8. Produit en fibres composites selon la revendication 7, dans laquelle le liant est un polymère organique.

9. Produit en fibres composites selon la revendication 7 ou la revendication 8, dans laquelle le liant est une substance dérivée du durcissement d'une composition polymère durcissable comprenant un polymère acrylique et un agent de liaison transversale contenant un groupement époxy.

10. Produit en fibres composites selon la revendication 9, dans laquelle le polymère acrylique est un homopolymère ou un copolymère comprenant des monomères dérivés d'au moins un monomère acrylique choisi dans les C_{1 à 4} alkyl (méth)acrylates.

11. Produit en fibres composites selon la revendication 9, dans laquelle le liant est une substance dérivée du durcissement d'une composition polymère durcissable comprenant un polymère acrylique basé sur le butyl acrylate et un agent de liaison transversale de résine époxyde.

12. Produit en fibres composites selon l'une quelconque des revendications précédentes, dans laquelle la répartition du liant dans le produit en fibres composites est telle que le pourcentage en poids du liant dans chaque zone de 1 mm³ du produit par rapport au poids total du produit dans cette zone ne dépasse pas 40% du pourcentage total en poids du liant dans le produit par rapport au poids total du produit.

13. Produit en fibres composites selon la revendication 12, dans laquelle la répartition du liant dans le produit de fibres composites est telle que le pourcentage en poids du liant dans chaque zone de 1 mm³ du produit par rapport au poids total du produit dans cette zone ne dépasse pas 30% du pourcentage total en poids du liant dans le produit par rapport au poids total du produit.

14. Produit en fibres composites selon l'une quelconque des revendications précédentes qui a une épaisseur de l'ordre de 3 à 15 mm.

15. Produit en fibres composites selon l'une quelconque des revendications précédentes, dans laquelle la charge du liant dans le produit est de l'ordre de 2 à 15% en poids par rapport au poids total du produit.

16. Produit en fibres composites selon l'une quelconque des revendications précédentes qui a une densité de l'ordre de 30 à 700 kg/m³.

17. Produit en fibres composites selon la revendication 16 qui a une densité située de l'ordre de 100 à 500 kg/m³.

18. Produit en fibres composites selon l'une quelconque des revendications précédentes qui a un cisaillement laminaire d'au moins 0,2 MPa.

19. Produit en fibres composites selon l'une quelconque des revendications précédentes qui est capable d'exercer une pression d'au moins 1,0 kgf/cm² lorsqu'une portion du produit ayant une épaisseur située entre 5 et 10 mm est compressée jusqu'à atteindre une épaisseur de 3 mm entre deux plaques et que le liant est retiré.

20. Produit en fibres composites selon la revendication 19 qui est capable d'exercer une pression de l'ordre de 1,5 à 4,0 kgf/cm² lorsqu'une portion du produit ayant une épaisseur située entre 5 et 10 mm est compressée jusqu'à atteindre une épaisseur de 3 mm entre deux plaques et que le liant est retiré.

21. Procédé pour la production d'un produit en fibres composites qui comprend l'imprégnation d'une masse de fibres comprenant une pluralité de fibres inorganiques avec un système de liaison liquide comprenant une substance liante et un liquide porteur, et le passage de la masse de fibres imprégnée à une étape de chauffage, caractérisée en ce que l'étape de chauffage fait intervenir un chauffage diélectrique.

22. Procédé selon la revendication 21, dans laquelle la masse de fibres imprégnée est maintenue sous compression pendant au moins une partie de l'étape de chauffage.

23. Procédé selon la revendication 21 ou la revendication 22, dans laquelle la masse de fibres qui est imprégnée est un produit multi-fibres dans lequel les fibres individuelles sont assemblées en un mat ou un tapis à faible densité.

24. Procédé selon la revendication 23 dans laquelle le produit multi-fibres a une épaisseur de l'ordre de 10 à 60 mm et une densité superficielle de l'ordre de 0,2 à 2,0 kg/m².

25. Procédé selon l'une quelconque des revendications 21 à 24, dans laquelle les fibres inorganiques ont une stabilité thermique pour des températures supérieures à 700°C.

26. Procédé selon la revendication 25, dans laquelle les fibres inorganiques sont des fibres céramiques.

27. Procédé selon la revendication 25 ou la revendication 26, dans laquelle les fibres inorganiques sont des fibres d'oxydes inorganiques polycristallins choisies dans le groupe constitué des fibres d'alumine, des fibres de mullite, des fibres d'aluminosilicate, des fibres d'aluminoborosilicate, des fibres de zircone et des fibres de titane.

28. Procédé selon la revendication 27, dans laquelle les fibres inorganiques sont des fibres d'alumine.

29. Procédé selon l'une quelconque des revendications 21 à 28, dans laquelle les fibres inorganiques sont de courtes fibres discontinues ayant une longueur allant de 1 à 10 cm et un diamètre moyen allant de 1 à 10 microns.

30. Procédé selon l'une quelconque des revendications 21 à 29, dans laquelle le système de liaison liquide comprend une substance liante organique et un liquide porteur organique ou aqueux qui est capable de dissoudre ou de disperser la substance liante organique.

31. Procédé selon la revendication 30, dans laquelle la substance liante organique est un polymère.

32. Procédé selon la revendication 30 ou la revendication 31, dans laquelle le système de liaison liquide comprend une dispersion d'une composition polymère durcissable comprenant un polymère acrylique et un agent de liaison transversale contenant un groupement époxy.

33. Procédé selon la revendication 32, dans laquelle le polymère acrylique est un homopolymère ou un copolymère comprenant des monomères dérivés d'au moins un monomère acrylique choisi dans les Ci à 4alkyl (méth)acrylates.

34. Procédé selon la revendication 32, dans laquelle le système de liaison liquide comprend une dispersion d'une composition polymère durcissable comprenant un polymère acrylique basé sur le butyl acrylate et un agent de liaison transversale de résine époxyde.

35. Procédé selon l'une quelconque des revendications 30 à 34, dans laquelle la dispersion est une dispersion aqueuse.

36. Procédé selon l'une quelconque des revendications 21 à 35, dans laquelle le système de liaison liquide comprend 0,5 à 50,0% en poids de substance liante et 50,0 à 99,5% en poids de liquide porteur.

37. Procédé selon la revendication 36, dans laquelle le système de liaison liquide comprend 1,0 à 5,0% en poids de substance liante et 95,0 à 99,0% en poids de liquide porteur.

38. Procédé selon la revendication 22, dans laquelle la totalité de l'étape de séchage/chauffage est réalisée tout en maintenant la masse de fibres imprégnée sous compression.

39. Procédé selon la revendication 22, dans laquelle la pression qui est appliquée au cours de l'étape de séchage/chauffage pour comprimer la masse de fibres imprégnée est de l'ordre de 5 à 500 KPa.

40. Procédé selon la revendication 39, dans laquelle la pression qui est appliquée au cours de l'étape de séchage/chauffage pour comprimer la masse de fibres imprégnée est de l'ordre de 5 à 200 KPa.

41. Procédé selon la revendication 21, dans laquelle le chauffage diélectrique est un chauffage par micro-ondes ou par fréquences radios.

42. Procédé selon la revendication 21, dans laquelle une combinaison de chauffage diélectrique et de chauffage conventionnel est utilisée au cours de l'étape de séchage/chauffage.

43. Procédé selon l'une quelconque des revendications 21 à 42, dans laquelle la masse de fibres imprégnée est chauffée à une température située entre 80 et 200°C au cours de l'étape de séchage/chauffage.

44. Procédé selon la revendication 43, dans laquelle la masse de fibres imprégnée est chauffée à une température située entre 100 et 170°C au cours de l'étape de séchage/chauffage.
